

May 6, 1941.

L. M. MYERS

2,241,215

LUMINESCENT SCREEN

Filed Nov. 26, 1938

*Fig. 1*



*Fig. 4*



*Fig. 2*



*Fig. 5*



*Fig. 3*



INVENTOR  
LEONARD MORRIS MYERS  
BY *Th. S. Grover*  
ATTORNEY

Patented May 6, 1941

2,241,215

# UNITED STATES PATENT OFFICE

2,241,215

## LUMINESCENT SCREEN

Leonard Morris Myers, Roseberry, Middlebrough, Yorkshire, England, assignor to Radio Corporation of America, a corporation of Delaware

Application November 26, 1938, Serial No. 242,501  
In Great Britain December 1, 1937

10 Claims. (Cl. 250—27.5)

This invention relates to the method of preparing luminescent screens as well as to provide improved screens for use, for example, in cathode ray tubes suitable for use for television reproduction on large screens and more particularly to television reproducer tubes in which reproduced pictures are built up on a "temperature radiating screen" by which expression is meant a picture reproducing screen which is scanned by a picture signal modulated cathode ray, elemental areas on the screen being so heated by the scanning bombarding ray, as to be raised to incandescence the pictures being thus obtained in the form of light from the heated elemental areas.

This invention embodies the new and improved screen in a television cathode ray reproducer tube with a temperature radiating screen comprising a highly refractory metallic layer supporting a layer of a highly refractory heater insulator which in turn carries a layer of a highly refractory metal in powdered form such as for example, a thin layer of lamp black on which is deposited a thin layer of fine tungsten powder. Now, as will be apparent, if ionized gas atoms are present in any quantity in the tube, the picture images will be adversely affected by these atoms bringing about a positive space charge with consequent gas focusing and it is, therefore, important that the degassing of the tube shall be as complete as possible. Lamp black is, however, extremely difficult to degas because of the large amount of absorbed gases it contains. The usual method of degassing the anode in an evacuated tube, is to bombard it with electrons (while pumping is proceeding) until the anode is hotter than any temperature it will reach in ordinary use. If, however, it is sought to apply this method to the above described temperature radiating screen, such large quantities of gas are emitted from the lampblack that, on bombardment at a high potential, serious cathodic sputtering occurs while, further, the anode or screen tends to disintegrate under the bombardment probably owing to oxidation of the carbon with the emitted oxygen from within its content. This is particularly noticeable in the case of the tungsten deposit which soon oxidizes during bombardment and forms the well known greenish tungstic acid.

The present invention overcomes these difficulties and according to the said invention, a cathode ray tube with a temperature radiating screen comprising a layer of lampblack refractory oxide or other material of poor heat conductivity and large gas content is characterized in that the said layer is carried upon a carrier member of tantalum or similar metal which, during degassing, has an electric current passed

therethrough so that it acts as a heater heating, by conduction, the material carrier thereon.

The invention is illustrated in the accompanying schematic drawing, in which

5 Figs. 1 to 3 show in different views one embodiment of the invention, while

Figs. 4 and 5 show elevation and plan views respectively of a modification of the embodiment of the invention shown in Figs. 1-3.

Referring first to Figures 1 to 3 which illustrate one way of carrying out this invention a temperature radiating screen is made of composite construction as follows: A tantalum carrier sheet is roughened in potassium hydroxide (KOH) and then slotted with a plurality of slits which start from two opposite edges of the sheet, each slit starting from one edge but stopping short of the other. In this way a series, zig-zag electrical path is created in the sheet this 10 path consisting of a series of strips which are side by side and lie in a plane. The slotted sheet is represented in Fig. 1 in which the carrier sheet as a whole is designated CS and the slits are designated CS<sup>1</sup> the strips between the slits being marked CS<sup>2</sup>. The two extreme end strips are left as shown at CS<sup>3</sup> to extend well beyond the rest of the opposite edges to facilitate electrical connection. Two mica plates MP<sup>1</sup> and MP<sup>2</sup> each with a large central rectangular window, are 15 placed one each side of the tantalum carrier CS the edges of these plates corresponding with the general edges of the tantalum carrier. Two nickel plates NP<sup>1</sup>, NP<sup>2</sup> shaped like the mica plates each with a rectangular window and of the same surface dimensions are placed outwardly of the mica discs. Bolt or rivet holes are provided in the nickel, mica, and tantalum members and these members are then clamped up in a pile by bolts B or rivets through these holes, 20 the tantalum (CS) being between two micas (MP<sup>1</sup> and MP<sup>2</sup>) and each mica being between the tantalum (CS) and one nickel (NP<sup>1</sup> or NP<sup>2</sup>). The bolts B or rivets should be insulated. The result is a frame in which the tantalum will then 25 be seen through the rectangular windows, the extended strip ends CS<sup>3</sup> of the tantalum projecting well beyond the micas and nickels. The tantalum in the windows is then carbonized on both sides with lampblack by holding the frame in a suitable flame—preferably a controlled benzine flame since this is found to give very pure lampblack. After thus coating with lampblack, tungsten powder is then shaken on through a muslin sieve. In place of using tungsten powder, a powder of other similar material—for example tantalum powder—could be deposited.

30 The frame, thus prepared, is then mounted in the tube in which it is to serve as screen and the tube then put on the pump and, as in the normal present day practice, subjected to a preliminary

baking while on the pump in order to remove water vapor from the glass envelope. While the oven is still hot and the tube is on the pump, a heating current is passed through the tantalum strip, this current being gradually increased until the maximum tantalum temperature—this should not exceed about 2,000° K. at which the lampblack will begin to evaporate—is reached. The tungsten or other surface of the screen will now glow dully owing to the high temperature gradient in the lampblack and if this procedure is continued the surface temperature will gradually increase until there is about 1,000° K. difference between it and the tantalum temperature. Maintenance of this condition for a few hours while under the pump will cause the lampblack to lose a great deal of its gas. Electron bombardment is then commenced, care being taken to ensure that the temperature of the lampblack does not exceed about 2200° K. as otherwise, owing to high vapor pressure, the carbon will rapidly evaporate. The final stage in the degassing is anode bombardment during which the screen surface is raised up to and finally beyond, maximum working temperature. This final stage will not now present any serious difficulties because, owing to the preliminary degassing operations, most of the gas has already been removed and there is therefore, no fear of deleterious cathode sputtering. This final stage, should, however, be accomplished with the tantalum strip carrier at its highest temperature in order that gas shall not be driven into the body of the screen.

The thickness of the films should be chosen with care and are somewhat critical. If the thicknesses are too great there will be insufficient heat from the tantalum reaching the outer surfaces; if they are too small, heat developed on the outermost surfaces by electron bombardment when the tube is in use will spread too easily to the tantalum and, by conduction therein, degrade the picture definition. A lampblack deposit of 0.25 mm. (or somewhat less) thick and a tungsten layer just thick enough to cover the lampblack are recommended.

The object of the lampblack is, of course, to keep the heat developed by electron bombardment when the tube is in use, in the tungsten or other surface material in which it is developed. In place of lampblack other suitable material, such as a refractory oxide, may be used. Suitable refractory oxides must possess high melting point and low vapor pressure, and for this reason MgO and ThO<sub>2</sub> are suitable examples.

Tantalum powder is somewhat preferred to tungsten powder because of its rather better emissivity the emissivity and temperature (in degrees K.) for tantalum being 80% and 2200 respectively for a brightness of 100 candles per square centimeter as against the figures of 70% and 2400 for tungsten, the corresponding figures for a black body being 100% and 2100.

Figures 4 and 5 show in sectional elevation and in plan view respectively an apparatus for a slightly modified way of carrying out the invention. In these figures MC is a molybdenum carrier on which is a layer of tungsten powder TP and which is mounted in close juxtaposition to a tungsten heater wire TW coated with aluminum silicate. This heater wire is between the carrier MC and a molybdenum sheet MS which is in turn carried by a support SP. Here the heating current is passed through the tungsten heater wire to facilitate the degassing operation.

I claim:

1. A luminescent screen comprising a thin planar sheet of high melting point metal, a layer of heat-insulating material deposited upon said planar sheet, said material having high melting point and low vapor pressure, and a layer of highly refractory powdered metal supported by said heat insulating material.
2. A luminescent screen comprising an electrical heating element, a layer of highly refractory heat insulating powder upon said element, and a planar layer of highly refractory metallic powder supported upon said heat insulating powder.
3. In the process of preparing a luminescent screen wherein is provided an electrical heating element, the steps of carbonizing the heating element to provide a highly refractory heat insulating layer thereon and depositing a highly refractory metallic powder upon the carbonized element.
4. In the process of preparing a luminescent screen wherein is provided an electrical heating element, the steps of carbonizing the heating element, depositing a highly refractory metallic powder upon the carbonized element, placing the carbonized element with its deposited powder within an envelope, evacuating the envelope, simultaneously passing current through the element to degas the carbonized element, and subsequently electronically bombarding the deposited powder to complete the degassing of the carbonized element.
5. In the process of preparing a luminescent screen, the steps of forming a planar electrical heating element coating the formed element with a layer of refractory heat-insulating material, and depositing a substantially planar layer of refractory metallic powder upon the layer of said material.
6. In the process of preparing a luminescent screen wherein is provided an electrical heating element, the steps of depositing a layer of refractory heat-insulating material upon the element, depositing a layer of refractory metallic powder upon the deposited layer of said material, placing the element with said deposited layer within an envelope, evacuating said envelope, simultaneously electrically heating said element and deposited layers, and subsequently electronically bombarding the deposited metallic layer to elevate the temperature of said deposited material to just below the temperature at which evaporation of said material takes place.
7. A luminescent screen comprising a highly refractory metal heater element, a layer of carbon on said element and a layer of highly refractory metallic powder supported upon said layer of carbon.
8. A luminescent screen comprising a planar tantalum sheet, a layer of carbon supported upon said tantalum sheet, and a layer of tantalum powder supported upon said layer of carbon.
9. A luminescent screen comprising a planar tantalum sheet, a layer of carbon supported upon said tantalum sheet and a layer of finely divided tungsten powder supported upon said layer of carbon.
10. A luminescent screen comprising a highly refractory metal heater element, a layer of highly refractory oxide on said heater element, and a substantially planar layer of finely divided highly refractory powder supported upon said layer of refractory oxide.